

## UNITED STATES PATENT OFFICE

2,528,605

## MOTOR FUELS

William Arthur Partridge and Harold John Alty,  
Sunbury-on-Thames, England, assignors to  
Anglo-Iranian Oil Company Limited, London,  
England, a British joint-stock corporation

No Drawing. Application September 20, 1946,  
Serial No. 698,406. In Great Britain September  
21, 1945

4 Claims. (Cl. 44—69)

1

The invention relates to the stabilisation of motor and aviation fuels containing anti-knock reagents.

The use of anti-knock reagents containing tetra-ethyl lead is widely known in the preparation of high quality fuels for use in internal combustion engines. In recent years there has been a growing demand for fuels showing a still greater resistance to knock, and particularly for aviation fuels. With a view to facilitate production of such fuels official specifications have appreciably relaxed the "lead tolerance," and the inclusion in such fuels of much larger proportions of anti-knock reagents is now permitted.

It is known that gasoline containing tetra-ethyl lead, and particularly aviation gasolines, which normally contain a higher proportion of the anti-knock reagent than motor gasolines, are liable to become unstable in storage, and to deposit a white precipitate containing lead. This instability becomes more marked as the lead content of the fuel rises, and thus the relaxation in lead tolerance allowed by official specifications accentuates the instability of such leaded fuels.

We have found that elemental sulphur, hydrogen sulphide, carbon disulphide, thiophene and dialkyl disulphides have a marked effect in producing instability, and that instability also appears to be promoted by certain olefins. Alkyl sulphides (thioethers) and mercaptans do not however appear to have any appreciable effect on the stability of a leaded fuel.

According to the invention, motor and aviation fuels containing tetra-ethyl lead are stabilised by the addition thereto of a minor proportion of a monocarboxylic acid or a salt or derivative thereof, but not including an ester thereof.

According to the invention moreover, monobasic fatty acids, or salts or derivatives of monobasic fatty acids, with the exception of esters, are employed as the inhibitors and in particular lead acetate, ammonium acetate and acetamide. Other mono-carboxylic acids, their salts and derivatives, with the exception of esters, may be used, however, whereas dibasic and hydroxy acids have no inhibiting properties.

The amount of the inhibitor required does not substantially exceed 0.01% by weight of the fuel, and in many cases satisfactory results are achieved when the fuel contains as little as 0.001% of the inhibitor.

2

The inhibitor may be incorporated in the fuel in a number of ways. It may be added for example to the finished fuel, or to any constituent of the fuel prior to blending, or to the anti-knock reagent, or it may be incorporated in the blending process or in the "leading" operation.

Lead salts are generally only sparingly soluble in motor and aviation fuels, and in order effectively to incorporate such salts of very low solubility in the fuel an excess of the salt may be added to the fuel, the exceedingly dilute solution formed being decanted. Or again the lead salt, and particularly lead acetate, may for example be added in the form of an alcoholic solution, since an apparent increase in the solubility of the salt in the fuel is thereby attained.

The following four non-inhibited fuels, each containing 5.5 MI.TEL/IG, were subjected to storage tests carried out in the dark at a temperature of 120° F. Fuel A was a commercial aviation fuel; fuel B was a sulphur-free iso-octane to which thiophene had been added in quantity sufficient to give the fuel a sulphur content of .005% by weight; fuel C was a sulphur-free iso-octane to which carbon disulphide had been added in quantity sufficient to give the fuel a sulphur content of .005% by weight; fuel D was a commercial aviation spirit.

The days required for the formation of precipitate with the non-inhibited fuels referred to were found to be as follows:

| Fuel | Trace | Medium | Heavy |
|------|-------|--------|-------|
| A    |       | 1      | 2     |
| B    | 5     | 6      | 8     |
| C    | 1     | —      | 2     |
| D    |       |        | 1     |

40 The time taken to form a medium or heavy precipitate is a measure of the instability to be expected in practice. The formation of a trace of precipitate is not considered to be of importance.

45 Of the following Examples, Example 1 shows the beneficial effect of monobasic fatty acids, their salts and derivatives, Example 2 shows the ineffectiveness of the esters of the fatty acids as inhibitors, Example 3 shows the effect of mixed salts of monobasic fatty acids, and Example 4 illustrates the effectiveness of mono-carboxylic

acids other than fatty acids, and the ineffectiveness of organic acids other than monocarboxylic acids.

## Example 1

| Proportions of particular Inhibitors added to the fuels denoted by the letters A, B, C and D | Days to form precipitate in the quantities denoted |          |       |
|----------------------------------------------------------------------------------------------|----------------------------------------------------|----------|-------|
|                                                                                              | Trace                                              | Moderate | Heavy |
| <i>Effect of Acetic Acid</i>                                                                 |                                                    |          |       |
| A+0.001% acetic acid                                                                         | >15                                                |          |       |
| <i>Effect of Acetic Anhydride</i>                                                            |                                                    |          |       |
| D+0.001% acetic anhydride                                                                    | 22                                                 | 26       | 26    |
| B+0.001% acetic anhydride                                                                    | 27                                                 | 41       | 46    |
| C+0.001% acetic anhydride                                                                    | 23                                                 |          |       |
| <i>Effect of Acetamide</i>                                                                   |                                                    |          |       |
| D+0.001% acetamide                                                                           | 15                                                 | 40       | 66    |
| B+0.001% acetamide                                                                           | 19                                                 | 36       | 66    |
| C+0.001% acetamide                                                                           | 14                                                 | 26       | 56    |
| <i>Effect of Ammonium Formate</i>                                                            |                                                    |          |       |
| A+0.001% ammonium formate                                                                    | 11                                                 |          | 18    |
| B+0.001% ammonium formate                                                                    |                                                    | 14       | 16    |
| C+0.001% ammonium formate                                                                    |                                                    |          | 14    |
| <i>Effect of Ammonium Acetate</i>                                                            |                                                    |          |       |
| A+0.005% ammonium acetate                                                                    | 9                                                  | 12       | 84    |
| A+0.001% ammonium acetate                                                                    | 18                                                 | 40       | >85   |
| A+0.001% ammonium acetate                                                                    | 12                                                 | 48       | 64    |
| B+0.001% ammonium acetate                                                                    | 18                                                 | 34       | 34    |
| B+0.001% ammonium acetate                                                                    | 34                                                 | 39       | 49    |
| C+0.005% ammonium acetate                                                                    | 27                                                 | 80       | 30    |
| C+0.001% ammonium acetate                                                                    | 9                                                  | 34       | 49    |
| <i>Effect of other acetates</i>                                                              |                                                    |          |       |
| D+excess zinc acetate                                                                        | 7                                                  | 14       | 23    |
| B+excess zinc acetate                                                                        | 1                                                  | 17       | 20    |
| B+excess cadmium acetate                                                                     | 6                                                  | 11       | 33    |
| B+excess sodium acetate                                                                      |                                                    | 1        | 23    |
| B+excess lead acetate                                                                        | 22                                                 | 25       | 23    |
| B+excess uranyl zinc acetate                                                                 | 2                                                  |          | 31    |
| C+excess lead acetate                                                                        |                                                    |          | 25    |
| <i>Effect of Ammonium Butyrate</i>                                                           |                                                    |          |       |
| A+0.001% ammonium butyrate                                                                   | 16                                                 |          | 21    |
| B+0.001% ammonium butyrate                                                                   | 6                                                  |          | 19    |
| C+0.001% ammonium butyrate                                                                   |                                                    |          | 19    |
| <i>Effect of Lead Palmitate</i>                                                              |                                                    |          |       |
| D+0.002% lead palmitate                                                                      |                                                    | 1        | 4     |
| C+0.002% lead palmitate                                                                      | 8                                                  |          | 9     |
| <i>Effect of Ammonium Stearate</i>                                                           |                                                    |          |       |
| B+excess ammonium stearate                                                                   | 8                                                  | 14       | 20    |
| C+excess ammonium stearate                                                                   |                                                    |          | 4     |
| <i>Effect of Lead Stearate</i>                                                               |                                                    |          |       |
| B+excess lead stearate                                                                       | 1                                                  | 7        | 50    |
| C+excess lead stearate                                                                       |                                                    | 1        | 36    |
|                                                                                              |                                                    |          | 10    |

## Example 2

| Proportions of esters of fatty acids added as inhibitors to the fuels denoted by the letters A, B, C and D | Days to form precipitate in the quantities denoted |          |       |
|------------------------------------------------------------------------------------------------------------|----------------------------------------------------|----------|-------|
|                                                                                                            | Trace                                              | Moderate | Heavy |
| B+0.001% methyl acetate                                                                                    | 6                                                  | 7        | 10    |
| C+0.001% methyl acetate                                                                                    |                                                    | 2        | 3     |
| D+0.001% methyl acetate                                                                                    |                                                    | 1        | 2     |
| B+0.001% Ethyl acetate                                                                                     |                                                    | 6        | 10    |
| C+0.001% Ethyl acetate                                                                                     |                                                    |          | 2     |
| D+0.001% Ethyl acetate                                                                                     |                                                    | 1        | 2     |
| B+0.05% Ethyl acetate                                                                                      | 2                                                  | 7        | 20    |
| C+0.05% Ethyl acetate                                                                                      |                                                    | 1        | 2     |
| D+0.05% Ethyl acetate                                                                                      |                                                    | 1        | 2     |
| B+0.001% amyl acetate                                                                                      | 5                                                  | 6        | 10    |
| C+0.001% amyl acetate                                                                                      |                                                    | 2        | 3     |
| D+0.001% amyl acetate                                                                                      |                                                    | 1        | 2     |
| A+0.001% phenyl acetate                                                                                    |                                                    |          | 3     |
| B+0.001% phenyl acetate                                                                                    |                                                    |          | 2     |
| C+0.001% phenyl acetate                                                                                    |                                                    |          | 3     |
| A+0.001% bornyl acetate                                                                                    |                                                    |          | 10    |
| B+0.001% bornyl acetate                                                                                    |                                                    |          | 6     |
| C+0.001% bornyl acetate                                                                                    |                                                    |          | 2     |
| A+0.001% vinyl acetate                                                                                     |                                                    |          | 12    |
| B+0.001% vinyl acetate                                                                                     |                                                    |          | 14    |
| C+0.001% vinyl acetate                                                                                     |                                                    |          | 3     |
| A+0.001% vinyl acetate                                                                                     | 2                                                  | 4        | 2     |
| B+0.001% vinyl acetate                                                                                     |                                                    |          | 6     |
| C+0.001% vinyl acetate                                                                                     |                                                    |          | 4     |

## Example 3

| Inhibitor                                         | No. of days for deposition of precipitate |        |       |
|---------------------------------------------------|-------------------------------------------|--------|-------|
|                                                   | Trace                                     | Medium | Heavy |
| Fuel C+0.001% lead acetate/ammonium acetate       | 7                                         |        | 18    |
| Fuel C+0.001% ammonium stearate/ammonium acetate  | 7                                         | 9      | 10    |
| Fuel C+0.001% ammonium stearate/zinc acetate      | 6                                         |        | 7     |
| Fuel C+saturated with lead palmitate/lead acetate | 6                                         |        | 7     |

## Example 4

| Inhibitor                              | No. of days for deposition of precipitate |        |       |
|----------------------------------------|-------------------------------------------|--------|-------|
|                                        | Trace                                     | Medium | Heavy |
| Fuel A+0.001% ammonium benzoate        |                                           |        | 8     |
| Fuel A+saturated with ammonium oxalate | 1                                         |        | 2     |
| Fuel A+saturated with ammonium citrate |                                           |        |       |
| Fuel B+0.001% ammonium benzoate        | 1                                         | 1      | 2     |
| Fuel B+saturated with ammonium oxalate | 2                                         | 3      | 5     |
| Fuel C+0.001% ammonium benzoate        | 1                                         | 2      | 5     |
| Fuel C+saturated with ammonium oxalate | 1                                         |        | 2     |
| Fuel C+saturated with ammonium citrate | 1                                         |        | 2     |

We claim:

1. A stabilised gasoline for use in internal combustion engines, said gasoline containing tetraethyl lead as anti-knock reagent and a small amount of an agent for preventing the formation of lead-containing precipitate, said agent being a compound of the formula  $\text{CH}_3\text{COR}$ , where R is a radical selected from the group consisting of  $\text{OH}$ ,  $\text{OCOCH}_3$ ,  $\text{NH}_2$ , and  $\text{ONa}$ .

2. A stabilised gasoline for use in internal combustion engines, said gasoline containing tetraethyl lead as anti-knock reagent and a small amount of an agent for preventing the formation of lead-containing precipitate, said agent being a compound of the formula  $\text{CH}_3\text{COR}$ , where R is a radical selected from the group consisting of  $\text{OH}$ ,  $\text{OCOCH}_3$ ,  $\text{NH}_2$ , and  $\text{ONa}$  and the small amount of the stabilising agent does not substantially exceed 0.01% by weight of the gasoline, and is not substantially less than 0.001%.

3. The method of stabilising gasoline for use in internal combustion engines, said gasoline containing tetraethyl lead as anti-knock reagent, which comprises mixing a small amount of an agent for preventing the formation of lead-containing precipitate with the gasoline, said agent being a compound of the formula  $\text{CH}_3\text{COR}$ , where R is a radical selected from the group consisting of  $\text{OH}$ ,  $\text{OCOCH}_3$ ,  $\text{NH}_2$ , and  $\text{ONa}$ .

4. The method of stabilising gasoline for use in internal combustion engines, said gasoline containing tetraethyl lead as anti-knock reagent, which comprises mixing a small amount of an agent for preventing the formation of lead-containing precipitate with the gasoline, said agent being a compound of the formula  $\text{CH}_3\text{COR}$ , where R is a radical selected from the group consisting of  $\text{OH}$ ,  $\text{OCOCH}_3$ ,  $\text{NH}_2$ , and  $\text{ONa}$ , and in which the amount of said agent does not substantially exceed 0.01% by weight of the gasoline, and is not substantially less than 0.001%.

WILLIAM ARTHUR PARTRIDGE,  
HAROLD JOHN ALTY.

## REFERENCES CITED

The following references are of record in the  
file of this patent:

## UNITED STATES PATENTS

| Number    | Name     | Date          | Number    |
|-----------|----------|---------------|-----------|
| 2,119,240 | Lyons    | Mar. 31, 1938 | 2,210,942 |
| 2,197,498 | Guthmann | Apr. 16, 1940 | 2,295,773 |
|           |          |               | 2,296,200 |

| Name            | Date           |
|-----------------|----------------|
| Lipkin          | Aug. 13, 1940  |
| Chenicek        | Sept. 15, 1942 |
| Cantrell et al. | Sept. 15, 1942 |

## FOREIGN PATENTS

| Country       | Date         |
|---------------|--------------|
| Great Britain | Apr. 8, 1940 |